

# UNITED STATES PATENT OFFICE.

GEORGE S. ENGLE, OF WASHINGTON, DISTRICT OF COLUMBIA, ASSIGNOR TO AMERICAN ELEMENTARY ELECTRIC COMPANY, OF WASHINGTON, DISTRICT OF COLUMBIA, A CORPORATION OF THE DISTRICT OF COLUMBIA.

## DOUBLE-COPPER-OXID BATTERY ELEMENT.

1,356,435.

Specification of Letters Patent. Patented Oct. 19, 1920.

No Drawing. Original application filed October 8, 1912, Serial No. 724,606. Divided and this application filed April 6, 1915. Serial No. 19,545.

To all whom it may concern:

Be it known that I, GEORGE S. ENGLE, a citizen of the United States, residing at Washington, in the District of Columbia, have invented new and useful Improvements in Double-Copper-Oxid Battery Elements, of which the following is a specification.

This invention relates to a double copper 10 oxid plate for use in primary batteries and other purposes, and is a division of my former application, Serial No. 724,606 filed October 8, 1912, allowed March 24, 1915, and the primary objects of the invention are to 15 provide a double copper oxid plate embodying in the main cupric oxid and a minimized quantity of cuprous oxid to form a battery element which will start electrolytic action without short circuiting or reducing the surface to cuprous oxid, and also 20 to produce a more durable and lasting element.

In forming the plate a bar of copper is heated to such temperature that when 25 sprayed with water blisters will be formed on the surface thereof. These blisters are then scraped off the bar in the form of copper flakes which are mainly black oxid of 30 copper or cupric oxid containing some pure metallic copper. These flakes are then suitably treated to eliminate any unctuous matter therefrom, such as oleaginous or greasy substances, by boiling the flakes in hot water, which latter step may be pursued without 35 in the least affecting or changing the desirable black oxid of copper properties of the flakes.

A binder is next prepared and consists of sugar, refined and clarified by bone black 40 and free of ultramarine blue, dissolved in water brought to the boiling point in the proportion of two parts sugar to one part of water. The flakes are thoroughly mixed with this binder and then pressed into compact form and shaped by any suitable means 45 and placed in a curing oven and subjected to heat. During this curing action the binder melts at 365° F.; between 400° and 420° F., the binder loses two molecules of 50 water and is converted into caramel, a very thick and black liquor. At a still higher temperature the binder yields combustible gases, etc., and the remaining portion of re-

siduum is one-fourth of its weight and in the form of charcoal. The heat of the curing 55 oven is carried up to 500° F.

The plate in the condition just specified is next placed in a baking oven where the temperature is about 1200° F. In this baking oven the charcoal residue of the binder 60 completely burns out without the least final residue, and the metallic copper is changed to cuprous oxid by the said high degree of heat. While the plate or product thus treated is red with heat it is immediately put into a 65 suitable press and compressed or forced into a hard, dense and strong mass of black oxid of copper and cuprous oxid. The plate or compressed mass is then taken from the press and allowed to cool in the air. 70

As hereinbefore stated, the resultant plate produced as explained will be found materially advantageous for the particular purpose for which it has been devised, as it will start electrolytic action without short 75 circuiting or reducing the surface to cuprous oxid and has a longer and more durable practical service than other plates having binders which cannot be wholly eliminated by heat and other means. 80

What is claimed is:

1. An element of an electric battery consisting of a copper oxid plate embodying black oxid of copper or cupric oxid in the main and a minimized quantity of cuprous oxid intimately mixed with the cupric oxid and entirely free of binder residuum. 85

2. An element of an electric battery consisting of a copper oxid plate embodying mainly cupric oxid and a minimum quantity of cuprous oxid in intermixed condition. 90

3. An element of an electric battery consisting of a plate composed of black oxid of copper or cupric oxid and red oxid of 95 copper or cuprous oxid mixed throughout the body of the plate.

4. An element of an electric battery consisting of a plate composed of cupric and cuprous oxids of copper held in compact 100 mass throughout the thickness of the plate without an additional binder.

5. An electrode for batteries composed of cupric oxid (CuO) and cuprous oxid (Cu<sub>2</sub>O). 105

6. An electrode for batteries formed of

cupric oxide flakes (CuO) and cuprous oxide (Cu<sub>2</sub>O).

7. An electrode for batteries formed of compressed cupric oxide in flake form and 5 cuprous oxide.

8. An electrode for batteries formed of compressed cupric oxide and cuprous oxide.

9. An electrode for batteries formed of cupric oxide and cuprous oxide in the form 10 of scales of appreciable size bonded together and compressed into a dense hard mass.

10. An electrode for batteries formed of

cupric oxide and cuprous oxide in the form of scales of appreciable size bonded and fused together in a dense, hard mass by the 15 application of heat and pressure.

In testimony whereof I have hereunto set my hand in presence of two subscribing witnesses.

GEORGE S. ENGLE.

Witnesses:

CHAS. S. HYER,

SADIE STANFORD WHITE.